

Patented Nov. 30, 1926.

## UNITED STATES PATENT OFFICE.

EDWARD W. HILL, OF CHICAGO, ILLINOIS, ASSIGNOR TO A. B. DICK COMPANY, OF CHICAGO, ILLINOIS, A CORPORATION OF ILLINOIS.

## STENCIL SHEET.

No Drawing.

Application filed December 3, 1923. Serial No. 678,163.

This invention relates generally to so-called "dry-process" stencil-sheets and particularly to sheets of the type employing as a coating constituent a material such as nitro-cellulose or other cellulose esters. The invention, which centers about the coating, as distinguished from the supporting base of yoshino or other porous fabric commonly employed in the art, has for its object to produce a material which shall, upon application to a supporting base, set quickly and completely impermeatize the sheet without repetition of the application; which shall be stable throughout an extended period of time and capable of receiving type-impressions without preliminary moistening or other treatment; which shall have a wide softening range and be therefore substantially unaffected by temperature changes, and which shall respond uniformly and clearly to the pressure of the type or stylus in the production of the desired stencil characters.

In carrying out the invention in an approved form, I first dissolve nitro-cellulose in a suitable volatile solvent such as ether-alcohol, amyl or ethyl acetate, acetone or a mixture containing two or more of these solvents. I then add a heavy, non-volatile oil (preferably one having lubricating properties), such as petroleum oil either with or without previous admixture of another solvent (such as a halogenated aliphatic hydrocarbon, an aliphatic or aromatic ester or the like), which will mix with both the solvents of the nitro-cellulose and the petroleum oil. I also add a tempering agent such as castor oil and, if found desirable, a fatty matter such as oleic or stearic acid or the like. I also prefer to employ a suitable plasticizing agent such as chlorinated naphthalene, acet-analid, or the like.

The order of addition of the ingredients to the solution may be greatly varied according to the character of the solvent used, the proportions desired and the temperature at which the mass is mixed. The mixture of solvents holds the nitro-cellulose, oils and plasticizing agent all in solution in the mass and of such mixture and such oils sufficient should be used to bring the compound to the proper consistency for coating the sheets of yoshino. Such coating may be effected in

the manner commonly practised, i. e., by drawing the yoshino over the surface of the 55 coating compound, which thereupon is taken up and absorbed by the fibres, after which the coated sheet may be hung to set as a result of the evaporation of the volatile solvents. As such evaporation proceeds, the 60 cellulose sets and occludes or encases, in a finely divided state, much of the petroleum oil along with some quantity of the vegetable oils and other constituents which are insoluble in and are non-solvents of the cellulose esters. The resulting coating on the paper is not, therefore, to be regarded as a 65 homogeneous mass but as one consisting of a solid or semi-solid mass which occludes or encases, in a finely divided state, a part of 70 the oils or oily masses, either liquid or semi-solid.

In making up my coating compound, I may, if desired, employ a suitable pigment or soluble dye-stuff, such, for example, as 75 carbon black, methylene blue and the like, serving not only to color the compound but, in the case of the pigment, to lend body to the compound. Also, as a bodying and toughening agent I may employ a suitable 80 gum, as resin, which is soluble in the mutual solvents but insoluble in petroleum oil. This gum resin may be either synthetic or natural. Coumarone resin of the synthetic group or gum sandarac of the natural group of 85 products will be found satisfactory. Finally, it is important to note that the invention is not limited to nitro-cellulose or cellulose acetate and, in fact, other cellulose esters may be employed instead. Consequently, to avoid limitation, I shall refer to this constituent herein by the term "chemically treated cellulose."

What I claim is:—

1. A stencil sheet coating which includes 95 a cellulose compound occluding or encasing a lubricant.
2. A stencil sheet coating which includes a cellulose compound occluding or encasing 100 a lubricant in a finely divided state.
3. A stencil sheet coating including nitro-cellulose occluding or encasing a lubricant.
4. A stencil sheet coating including nitro-cellulose occluding or encasing a hydrocarbon oil. 105
5. In a type-impressible stencil-sheet, an

- open, porous base having a coating including a cellulose compound and a hydrocarbon oil.
6. In a type-impressible stencil-sheet, an open, porous base having a coating including a cellulose compound and a heavy, hydrocarbon oil.
7. In a type-impressible stencil-sheet, an open, porous base having a coating including a cellulose compound and a non-volatile hydrocarbon oil.
8. In a type-impressible stencil-sheet, an open, porous base having a coating including a cellulose compound and a heavy, non-volatile hydrocarbon oil.
9. In a type-impressible stencil-sheet, an open, porous base having a coating including a cellulose compound, a tempering agent and a non-volatile oil.
10. In a type-impressible stencil sheet, an open, porous base having a coating including a cellulose compound, a tempering agent and a heavy, non-volatile oil.
11. In a type-impressible stencil-sheet, an open, porous base having a coating including a cellulose compound, a tempering agent and a non-volatile hydrocarbon oil.
12. In a type-impressible stencil sheet, an open, porous base having a coating including a cellulose compound, a tempering agent and a plasticizing agent.
13. In a type-impressible stencil sheet, an open, porous base having a coating including a cellulose compound, a tempering agent, a plasticizing agent, and a non-volatile oil.
14. In a type-impressible stencil-sheet, an open, porous base having a coating including a cellulose compound, a tempering agent, a plasticizing agent, and hydrocarbon oil.
15. In a type-impressible stencil-sheet, an open, porous base having a coating including a cellulose compound, a tempering agent, a plasticizing agent, and heavy, hydrocarbon oil.
16. In a type-impressible stencil-sheet, an open, porous base having a coating including a cellulose compound, a tempering agent, a plasticizing agent and a heavy, non-volatile hydrocarbon oil.
17. In a type-impressible stencil-sheet, an open, porous base having a coating including a cellulose compound, castor oil, a plasticizing agent and hydrocarbon oil.
18. In a type-impressible stencil-sheet, an open, porous base having a coating including a cellulose compound, castor oil, a plasticizing agent and heavy, hydrocarbon oil.
19. In a type-impressible stencil-sheet, an open, porous base having a coating including a cellulose compound, a tempering agent, a non-volatile oil and fatty matter.
20. In a type-impressible stencil-sheet, an open, porous base having a coating including a cellulose compound, a tempering agent, a non-volatile oil, a plasticizing agent and fatty matter.
21. In a type-impressible stencil sheet, an open, porous base having a coating including a cellulose ester, a tempering agent, and chlorinated naphthalene.
22. The process of producing a type-impressible stencil-sheet which consists in coating an open, porous base with chemically treated cellulose in solution and another material possessing lubricating properties occluded or encased in such cellulose.
23. The process of producing a type-impressible stencil-sheet which consists in coating an open, porous base with chemically treated cellulose in solution and another material possessing lubricating properties occluded or encased in such cellulose in a finely divided state.
24. The process of producing a type-impressible stencil-sheet which consists in coating an open, porous base with chemically treated cellulose in solution, another material possessing lubricating properties occluded or encased in such cellulose, and a plasticizing agent.
25. The process of producing a type-impressible stencil-sheet which consists in coating an open, porous base with chemically treated cellulose in solution, another material possessing lubricating properties occluded or encased in such cellulose in a finely divided state, and a plasticizing agent.
- This specification signed and witnessed this 28th day of November, 1923.
- EDWARD W. HILL.